

## UNITED STATES PATENT OFFICE

RENÉ CLAVEL, OF BASEL-AUGST, SWITZERLAND

## TREATMENT OF ARTIFICIAL SILKS

No Drawing. Application filed May 27, 1927, Serial No. 194,859, and in Germany September 17, 1926.

This invention relates to processes for weighting artificial silks.

As is known, the weighting of artificial silks presents very considerable difficulties, owing 5 to the fact that artificial fibres of cellulose or cellulose derivatives are very sensitive to the action of weighting agents and in many cases to the action of water. The many passages 10 of the hanks or fabrics through a series of baths containing separately the individual weighting agents, as is customary in natural silk weighting processes and through the intermediate washing or neutralizing baths, which are necessary between the actual 15 weighting baths, are particularly unfavorable for artificial silks. In the case of artificial silks made from cellulose esters, apart from the injury to the fibres, a saponification of the cellulose esters often occurs, by 20 which the silk suffers and frequently becomes useless. The aim of artificial silk weighting must therefore be to effect the weighting in as few baths as possible.

I have now found that very successful 25 weighting of artificial silks may be obtained by employing two or more weighting agents in one bath or by employing successive weighting baths (impregnating and precipitating baths) without intermediate washing or neutralizing, the fibre and/or at least one 30 of the baths having added or applied thereto a substance adapted to hinder premature precipitation, i. e. precipitation either in the bath or at the surface of the fibre.

Such substances may be mineral or organic acids, acid salts or salts having an acid 35 reaction or protective colloids such as glue, gelatine, albumen or the like. If desired the substance used to hinder premature precipitation may itself be a weighting substance. Thus for example aluminum sulphate has a 40 very pronounced acid reaction and may act at the same time as a weighting agent.

When employing two or more weighting 45 agents in one bath according to the present invention, for example metal compounds (especially compounds of tin and zinc) and salts, e. g. phosphates, sulphates, silicates and the like or acids such as phosphoric acid and 50 also if desired tanning substances, the bath

or two or more of such baths may be made up with an acid, an acid salt or protective colloid or other agent adapted to hinder precipitation or with a mixture of such agents. The goods may then be passed directly through the bath or two or more of such baths, or if desired an acid, acid salt or protective colloid or other agent adapted to hinder premature precipitation or a mixture thereof may also be applied to the goods 55 themselves prior to passage through the bath or baths. 60

Again when employing successive weighting baths (for example baths of tin or zinc compounds and of salts such as phosphates, sulphates, for instance of alumina, or silicates, or of acids, for example phosphoric acid) one or more of the said agents adapted 65 to hinder precipitation may be applied to the goods or to at least one of the baths or both to the goods and at least one of the baths and the goods passed successively through the baths without intermediate washing or 70 neutralizing.

By means of the invention the weighting 75 of artificial silks can be effected by passing through only a comparatively small number of baths, neutralizing and washing being eliminated, or even through a single bath only, and further the hanks, fabrics or other goods 80 need only remain in the baths a very short time to obtain the required weighting.

In order to obtain a better fixation of the weighting agents and in certain cases in order to remove excess of acid, the materials 85 after weighting and preferably after squeezing may be treated in a bath having an alkaline reaction, for example a solution of ammonium carbonate, to which if desired dye-stuffs which contain tanning substances, such as haematein, may be added. 90

The invention is applicable to the weighting of all artificial silks made from cellulose or cellulose derivatives, for example acetyl cellulose silks, viscose silks, Chardonnet silks and cuprammonium silks. 95

The following examples may be given in illustration of the invention, it being understood that they are in no way limitative and 100

can be varied widely without departing from the spirit of the invention.

*Example 1*

5 An acetyl cellulose fabric woven in the piece is passed through a finishing machine in which it passes first through a bath of 5 litres of a 10% aqueous albumen solution containing 50 grams of ammonium carbonate. The 10 travelling fabric is squeezed out on the same machine and passes on into a second bath composed of a 4 per cent tin chloride solution containing 10 per cent phosphoric acid per litre. It is dried and dyed with direct 15 dyestuffs.

*Example 2*

Acetyl cellulose artificial silk in any form is soaked in a 5% solution of aluminum acetate in the container of a centrifuge. The 20 solution is run off and the goods centrifuged after which a solution containing 4% of tin chloride and 10% phosphoric acid is introduced. The goods may then again be 25 centrifuged, treated with ammonium carbonate solution and dried and if desired dyed with direct dyestuffs.

*Example 3*

30 10 litres of the weighing bath contain:

200 grams zinc chloride.  
100 grams sulphate of aluminium.  
400 grams anhydrous tin chloride.

35 The textile goods are passed through the bath, squeezed out, and then led through a 3 per cent solution of sodium phosphate, dried and dyed.

*Example 4*

40 A fabric consisting wholly or partly of acetyl cellulose artificial silk, e. g. a crêpe de chine fabric, is led in full width through a 1% aqueous solution of phosphoric acid containing 12 grms. of glue per litre. The fabric is 45 then carried directly through four tin chloride baths containing tin tetrachloride solution of 35° Bé. strength and is thereafter squeezed and led first into a 10% monosodium phosphate bath and then into a 6% disodium phosphate bath. After the alkaline phosphate bath the fabric is hydro-extracted and 50 may if desired be finally treated in a water-glass solution of 1° Bé. containing 1 gm. of soap per litre.

*Example 5*

An artificial silk fabric is passed on a finishing machine through a 10 litre bath containing 400 grms. of zinc chloride and 100 grms. 60 of formic acid. The fabric is then passed directly without washing through a 6-8% aqueous solution of monosodium phosphate. The artificial silk may then be squeezed, passed through a 5% solution of ammonium 65 carbonate and dried.

*Example 6*

Acetyl cellulose artificial silk in the form of hanks is immersed for a short time in a 1% solution of monochloracetic acid. The treated hanks are brought into a bath containing 70 tin tetrachloride of 35° Bé. and are then stretched and allowed to remain in the air for a short time. The procedure may be repeated if desired. The hanks are well centrifuged and entered for a short time into a 15% solution of monosodium phosphate. They are 75 squeezed or hydro-extracted and if desired after a short washing may be given a final treatment in a 1% solution of waterglass containing soap at 40° C. 80

Goods of acetyl cellulose or the like weighted according to the invention are increased in volume considerably and have a much increased affinity for direct dyeing sulphonated dyestuffs, which ordinarily dye acetyl cellulose little or not at all. Owing to the relatively short duration of treatment in the baths their strength is substantially unimpaired. 85

Owing to the omission of intermediate washing or neutralization, diluted solutions of the weighing agents or of transformation products thereof resulting from neutralization are not obtained and in consequence the special installations and considerable expense usually entailed in the recovery of such agents or products are avoided. 90

An additional advantage accrues when a treatment of the goods with an acid substance is carried out prior to the weighting, it being found that a more intensive and more uniform absorption of the weighting agents is brought about and the duration of the whole weighting process is considerably reduced. 100

What I claim and desire to secure by Letters Patent is:

1. Process for weighting artificial silks, comprising treating them with a plurality of weighting agents without intermediate washing or neutralization, at least one substance being employed which is adapted to hinder premature precipitation. 110

2. Process for weighting acetyl cellulose artificial silks comprising treating them with a plurality of weighing agents without intermediate washing or neutralization, at least one substance being employed which is adapted to hinder premature precipitation. 115

3. Process for weighting artificial silks, comprising treating them with a plurality of weighting agents in one bath, which contains at least one substance adapted to hinder premature precipitation. 120

4. Process for weighting artificial silks, comprising treating them with a plurality of weighting agents in one bath, which contains a substance having an acid reaction to hinder premature precipitation. 125

5. Process for weighting artificial silks 130

- comprising treating them with a plurality of weighting agents in one bath, in the presence of a protective colloid and a substance having an acid reaction to hinder premature precipitation.
6. Process for weighting artificial silks, comprising treating them with a plurality of weighting agents in one bath, which contains an acid to hinder premature precipitation.
10. Process for weighting artificial silks, comprising treating them with a substance having an acid reaction and then with a plurality of weighting agents in one bath, which contains a substance having an acid reaction to hinder premature precipitation.
15. Process for weighting artificial silks, comprising treating them with an acid and then with a plurality of weighting agents in one bath, which contains an acid to hinder premature precipitation.
20. Process for weighting artificial silks, comprising treating them with a plurality of weighting agents in one bath, which contains a substance having an acid reaction to hinder premature precipitation, and thereafter treating with an alkaline solution.
25. Process for weighting artificial silks, comprising treating them with a plurality of weighting agents in one bath, which contains a substance having an acid reaction to hinder premature precipitation, and thereafter treating with ammonium carbonate solution.
30. Process for weighting artificial silks, comprising treating them with a plurality of weighting agents in one bath, which contains an acid to hinder premature precipitation, and thereafter treating with an alkaline solution.
35. Process for weighting artificial silks, comprising treating them with a plurality of weighting agents in one bath, which contains an acid to hinder premature precipitation and thereafter treating with an alkaline solution.
40. Process for weighting artificial silks, comprising treating them with an acid and then with a plurality of weighting agents in one bath, which contains an acid to hinder premature precipitation and thereafter treating with an alkaline solution.
45. Process for weighting acetyl cellulose artificial silks comprising treating them with a plurality of weighting agents in one bath, which contains at least one substance adapted to hinder premature precipitation.
50. Process for weighting acetyl cellulose artificial silks, comprising treating them with a plurality of weighting agents in one bath, which contains an acid to hinder premature precipitation.
55. Process for weighting acetyl cellulose artificial silks, comprising treating them with an acid and then with a plurality of weighting agents in one bath, which contains an acid to hinder premature precipitation.
60. Process for weighting acetyl cellulose artificial silks, comprising treating them with a plurality of weighting agents in one bath, which contains a substance having an acid reaction to hinder premature precipitation, and
- thereafter treating with an alkaline solution.
17. Process for weighting acetyl cellulose artificial silks, comprising treating them with a plurality of weighting agents in one bath, which contains a substance having an acid reaction to hinder premature precipitation and thereafter treating with ammonium carbonate solution.
18. Process for weighting acetyl cellulose artificial silks, comprising treating them with an acid and then with a plurality of weighting agents in one bath, which contains an acid to hinder premature precipitation and thereafter treating with an alkaline solution.
19. Process for weighting acetyl cellulose artificial silks comprising treating them with a plurality of weighting agents in one bath, in the presence of a protective colloid and a substance having an acid reaction to hinder premature precipitation.
- In testimony whereof I have hereunto subscribed my name.
- RENE CLAVEL.